

Oct. 30, 1928.

1,689,693

C. SHAPLEY

FLOTATION PROCESS

Filed Oct. 13, 1927



Inventor  
Cooper Shapley  
by  
J. H. Maxwell  
his Attorney

Patented Oct. 30, 1928.

## UNITED STATES PATENT OFFICE.

COOPER SHAPLEY, OF BISHOP, CALIFORNIA.

## FLOTATION PROCESS.

Application filed October 13, 1927. Serial No. 225,907.

The invention relates to a process of separating particles of solid matter from one another by means of flotation, and it is a general object of my invention to provide a flotation process which is practical, simple and inexpensive to carry out, and by which it is possible to treat particles of material which have heretofore never been successfully handled by flotation processes.

My invention provides, primarily, for the successful separation of solid particles by flotation in which soap is the sole medium or reagent used. Essentially, the invention provides for contacting of ground particles of the material to be separated with a soap solution, whereby those particles having an attraction for soap are contacted with the solution to become coated or filmed by the soap, and then bringing the soap-filmed particles to the surface of a body of liquid, say water, where they will remain, and from which they can be removed.

I am aware that soap has been suggested and tried in various ways and under various conditions in the art of separation of materials by flotation. However, I believe that all prior uses and proposals for using soap in this art have been quite far removed from the principles and spirit of my present invention. In the earlier processes referred to, the soap has been used as a frothing agent, and in connection with oils, acids and other substances, or so as to have a chemical reaction upon the particles contacted thereby. So far as I am aware, it has not been heretofore proposed to employ a soap solution as the sole agent of flotation and for separating particles with which the soap does not chemically react.

The art of mineral separation by flotation, although well established and developed, has heretofore been more or less limited commercially to the concentration of minerals having a metallic lustre. This is because the flotation methods which have been commercially practical have been inoperative or impractical on minerals lacking metallic lustre.

It is an object of my invention to provide a commercially practical flotation process which will include mineral lacking metallic lustre.

Another object of my invention is to provide a flotation process which can be successfully carried out on particles of matter materially larger than can be successfully handled by the usual flotation methods.

A further object of my invention is to provide a flotation process in which the separation takes place quickly in the flotation machine.

It is a primary object of my present invention to provide a process of flotation which makes possible the practical separation of particles with the use of soap alone. In carrying out this object, I provide a process which is extremely simple and inexpensive, and eliminates chemical reactions and complications such as have been present in flotation processes heretofore proposed.

As previously noted, one of the principal objects of the invention is to provide a method or process of flotation by which it is possible to successfully separate particles which have never heretofore been successfully separated by flotation, for example, calcium minerals and many minerals lacking in metallic lustre.

My present invention involves numerous other objects and features which, with those above mentioned, will be best and more fully understood from the following detailed description of a typical application and means for carrying out the invention, throughout which description I will refer to the accompanying drawing showing diagrammatically an arrangement of apparatus that may be employed in carrying out the particular application of the invention which will be described.

While the invention is useful, generally, in the separation of materials or minerals by flotation, it is particularly adapted for separating or recovery of materials which do not chemically react with a soap solution, such, for example, as fluorite, rutile and corundum. It is to be understood, of course, that the invention is not intended to be limited to treatment of the particular materials given as examples. Experience has shown that the methods herein described will not float particles of certain materials, examples of which are quartz, felspar, and mica, but, as above noted, the invention has been found very successful in separating ores which could not be successfully treated by the flotation processes heretofore proposed.

For example, I may treat ore bearing fluorspar (calcium fluoride) and closely approach a complete separation of the fluorspar from the gangue or quartz. Fluorspar, which is a mineral used in various arts, such as enameling, steel manufacture, glass manufacture,

etc., is found in crystalline form with quartz or other silicates, and it has not been practical by the flotation processes heretofore proposed to effectively separate this material from the 5 undesired substances.

- In applying my invention to the handling of ore for the separation of certain values therefrom, the ore is first ground by any suitable means, for instance, in a mill 10. My 10 invention is in many cases superior over most processes of flotation in that it will successfully handle ore in a comparatively coarse state. In the case of ore bearing fluorspar, I have obtained successful separation upon 15 grinding the ore to pass a screen of about 10 mesh. In practice, it may be desirable to grind the ore somewhat finer, but it is unnecessary in most cases for it to be any finer than will pass a screen of 60 mesh.
- 20 The ore, after grinding, preferably is drained of the excess water; for instance, it may be passed from the grinder 10 into a dewatering tank from which it is withdrawn from the water by a scraper belt 12. The dewatering tank, shown in the drawings, has an inclined part 13 over which the ground ore is scraped from the tank by the scraper 12. This incline allows the excess water to drain back into the tank. The primary object of 25 dewatering the ground ore is to avoid dilution of the soap solution to which the ore is next passed. The ore delivered from the dewatering tank 11 in the damp or partly wet condition is delivered to a treatment tank 30 14 containing a soap solution. The ore is preferably introduced into the tank 14 so that it is submerged in the soap solution and thus thoroughly contacted with the solution. It is preferred to make a colloidal soap solution 35 from sodium or potassium soaps and water, and I make a fairly dilute or weak solution, say for example, a solution containing about one per cent or less of soap. I have found that the solution may be even 40 weaker than this; in fact, from experience, I am led to believe that there is no critical strength of solution necessary for the successful operation of the invention. It seems merely necessary to have sufficient soap 45 present in the solution so that the particles treated are contacted with soap to hold or retain it if possessing the proper characteristics. When I use the term "weak soap solution", I mean a solution of about the character 50 mentioned above. The quantity of soap required per ton of ore varies. In some cases, I have obtained satisfactory results with as 55 low as two pounds of soap per ton, while in other cases, I have obtained the best results with about ten pounds of soap per ton. As 60 an example, I may state that I have carried out the process on a commercial scale on an ore bearing fluorspar using about four pounds of soap per ton.

65 Referring to ore bearing fluorspar, which

I am citing as an example, the contacting of the ore with the soap solution results in the coating or filming of the fluorspar particles with soap. The fluorspar has an attractive or adsorptive quality for the soap particles 70 which causes the soap particles to apply themselves to the fluorspar particles. My observations indicate that the soap particles merely apply or coat themselves to the fluorspar particles and that there is no chemical reaction between the two. I have found it 75 advantageous to apply the ore to the treatment tank 14 with as little agitation as possible to keep the soap solution quiet and thus avoid decomposition of the soap. It is to 80 be understood that the soap solution may be renewed or suitably maintained at the desired strength so that the process may be carried out continuously.

The soap solution referred to may be initially produced outside of the treatment tank 14 or produced in such tank by supplying thereto ingredients which will form a soap solution of the desired character.

It will be understood that the strength of 90 the soap solution is to be such as will satisfy the soap absorbing properties of the particles to be separated.

The ore, after having been subjected to the soap solution to allow the particles to thoroughly contact with the soap solution, is removed from the treatment tank 14 as by a belt scraper 15. The treatment tank may be provided with an inclined part 16 over which the ore is scraped from the tank, thus allowing 100 the solution to drain back into the tank. This method of removing the ore from the treatment tank provides for the desired removal of the ore with a minimum of agitation which, as above pointed out, is preferably to 105 be avoided. This manner of removing the treated ore from the treatment tank is to separate the excess or unused soap solution from the ore, and, if it is found that the separation is insufficient, the ore, after leaving the treatment tank, may be given a water wash; for instance, it may be passed through 110 a washing tray 17. The removal of excess soap is desired as the soap may reduce the surface tension of the water on which the 115 coated particles are to be floated. I may state at this point that the soap particles, when once applied to the fluorspar particles, adhere to and permanently coat or film the fluorspar so that they are not removed by 120 ordinary water washing.

The ore, after thus being freed from the soap solution, is handled to bring the fluorspar particles to the surface of a body of water free from any reagent which will act 125 to decompose the absorbed soap, coating the separated particles. This treatment may be carried out by agitation in an ordinary flotation machine 18. The soap bearing fluorspar particles, upon reaching the surface of the 130

body of water, will remain on the surface and will accumulate in the form of a scum. The accumulation of particles on the surface is, in fact, a scum and is not a froth as is the case with the usual methods of flotation. It will be obvious that the fluorspar particles accumulating on the surface of the body of water as a scum may be removed in any suitable manner; for instance, they may be allowed to flow or fall over an overflow edge provided for that purpose. The separated or concentrated fluorspar thus obtained may be received and thereafter handled in any suitable manner.

15 I have found by actual operation that it is not necessary to water wash the pulp or minerals after contacting them with the soap solution. By using sufficient water in the flotation machine, separate water washing is unnecessary, as the bulk of water in the machine is constantly changing and carrying away tailings. I have found that this condition dilutes the soap solution so much that the pulp needs no washing after being contacted.

Having thus described the invention, what I claim is:

1. The process of separating finely divided particles by flotation comprising contacting the particles with a soap solution which does not chemically react with the particles, and then bringing the particles to the surface of a body of water free from any reagent which would decompose the soap.

35 2. The process of separating finely divided

particles by flotation comprising contacting the particles quietly with a soap solution which does not chemically react with the particles, and then bringing the particles to the surface of a body of water free from any reagent which would decompose the soap.

3. The process of separating finely divided particles by flotation comprising contacting the particles with a soap solution of a strength to satisfy the soap absorbing properties of the particles and then bringing the particles to the surface of a body of liquid free from any reagent which would decompose the soap.

4. The process of separating finely divided particles by flotation comprising contacting the particles with a soap solution, separating the particles from the solution including washing the particles with water, and then bringing the particles to the surface of a body of liquid free from any reagent which will decompose the soap.

5. The process of separating finely divided particles by flotation comprising contacting the particles with a soap solution which does not chemically react with the particles, separating the soaped particles from the solution including washing them with water, and then bringing the soaped particles to the surface of a body of liquid free from a reagent which will decompose the soap.

In witness that I claim the foregoing I have hereunto subscribed my name this 8th day of October, 1927.

COOPER SHAPLEY.